

# United States Patent [19]

Koppenaal et al.

[11] 3,920,490

[45] Nov. 18, 1975

[54] THERMALLY PROCESSED STEEL

[75] Inventors: **Theodore J. Koppenaal**, Newport Beach; **Richard P. Sernka**, Irvine, both of Calif.

[73] Assignee: **Ford Motor Company**, Dearborn, Mich.

[22] Filed: **Dec. 7, 1973**

[21] Appl. No.: **422,947**

Related U.S. Application Data

[63] Continuation-in-part of Ser. No. 172,808, Aug. 8, 1971, abandoned.

[52] U.S. Cl. .... **148/12.4**; 148/125; 148/143; 148/144

[51] Int. Cl. .... **C21D 6/04**; C21D 7/02; C21D 1/22

[58] Field of Search ..... 148/2, 3, 12, 12.4, 13, 148/14, 134, 143, 144, 12.3, 125

[56] References Cited

UNITED STATES PATENTS

|           |         |                  |         |
|-----------|---------|------------------|---------|
| 3,288,657 | 11/1966 | Morita et al.    | 148/143 |
| 3,316,129 | 4/1967  | Token et al.     | 148/135 |
| 3,370,994 | 2/1968  | Konkol           | 148/142 |
| 3,378,367 | 4/1968  | Friis et al.     | 75/128  |
| 3,385,740 | 5/1968  | Baggstrom et al. | 148/136 |

3,488,231 1/1970 Zackay et al. .... 148/12

OTHER PUBLICATIONS

Transactions of the Metallurgical Society of AIME, Vol. 224, Dec. 1962, pp. 1212-1221.

Transactions of ASM, Vol. 61, 1968, pp. 26-36.

Primary Examiner—C. Lovell

Attorney, Agent, or Firm—Joseph W. Malleck; Keith L. Zerschling

[57] ABSTRACT

This invention relates to a process for producing an austenitic steel with a combination of high strength and high elongation by a process involving thermal manipulation. No mechanical deformation is essential but can contribute some additional benefits. The process taught by this invention is applicable to any steel in which the  $M_s$  is well below the lowest anticipated service temperature, the austenite reversion temperature is substantially below the point at which the austenite recrystallizes, and where the  $M_d$  is increased by the thermal manipulation. This invention involves repeated thermal cycling between austenite and martensite.

7 Claims, 12 Drawing Figures

FIG. 1



INVENTORS  
RICHARD P. SERNKA  
THEODORE J. KOPPENAAL  
BY  
John R. Faulkner  
Thomas H. Oster  
ATTORNEYS



FIG.4



FIG.5



FIG.6



INVENTORS

RICHARD P. SERNKA  
THEODORE J. KOPPENAA

BY

John R. Faulkner  
Thomas H. Oster  
ATTORNEYS

FIG.7



FIG.8



FIG.9



INVENTORS

RICHARD P. SERNKA  
THEODORE J. KOPPENAAL  
BY

*John R. Faulkner  
Thomas H. Oster*  
ATTORNEYS

FIG. 10

INVENTORS  
RICHARD P. SERENKA  
THEODORE J. KOPPENAAAL  
BY  
John R. Faulkner  
Thomas H. Oster  
ATTORNEYS

FIG. II



INVENTORS  
RICHARD P. SERENKA  
THEODORE J. KOPPENAAL  
BY  
John R. Faulkner  
Thomas H. Oster  
ATTORNEYS

FIG. 12



INVENTORS  
 RICHARD P. SERNKA  
 THEODORE J. KOPPENAAL  
 BY  
 John R. Faulkner  
 Thomas H. Oster  
 ATTORNEYS

## THERMALLY PROCESSED STEEL

## CROSS-REFERENCE TO RELATED APPLICATION

This application is a continuation-in-part of our co-pending application Ser. No. 172,808, filed Aug. 8, 1971, now abandoned and having the same title as the present application.

## BACKGROUND OF THE INVENTION

The current invention permits the production of austenitic steels having a combination of high strength and high elongation without the necessity of deforming the steel to obtain these properties. Zackay and Parker recently were awarded U.S. Pat. No. 3,488,231, Jan. 6, 1970, for developing a class of high strength and high elongation steels wherein these mechanical properties are achieved by the use of a deformation cycle during the processing. This prior art method can best be characterized as a warm plastic deformation cycle wherein the austenite is strained by reduction in thickness up to 80% and by working at temperatures in the range of 800°-1200°F; the yield strength can be increased up to about 200 ksi by this method. Since the high elongation values resulted from the control of the austenite to martensite phase transformation, Zackay and Parker labeled the phenomenon "TRIP", which is abbreviated from the words "Transformation Induced Plasticity".

This invention provides an alternative to this prior art method by avoiding the requirement for large equipment needed to impose strain and by avoiding the limitation to thin sections. Thus, under ambient temperature service conditions, there will be a transformation from strained austenite to martensite rendering an increase in strength and ductility for the particular steel, but this will have been brought about by a unique thermal cycling, rather than by mechanical treatment.

According to Zackay and Parker and other related prior art, the thermal martensite start temperature,  $M_s$ , must be below ambient while only the deformation or martensite start temperature,  $M_d$ , is above ambient. Warm plastic deformation will then harden the austenite and reportedly promotes carbide precipitation, thus altering the matrix chemistry. This combination appropriately adjusts the  $M_s$  and  $M_d$  with the ambient temperature condition occurring between them. When alloys, so processed, are stressed at room temperature, the onset of plastic strain is accompanied by transformation from cold worked austenite to martensite; the amount (volume) transformed being partially dependent upon the amount of plastic strain. This transformation to martensite strengthens the mass locally, shifting the region of strain. This has the effect of producing extensive uniform strain (elongation) in the volumes stressed in tension. Strength is primarily increased by cold working the austenite and the high elongation is a result of the shift in  $M_d$  to above room temperature.

In contrast, this invention uses steels which have the starting  $M_s$  and  $M_d$  both below ambient or room temperatures; but, surprisingly, the method herein permits the adjustment of the  $M_s$  and  $M_d$  solely by thermal excursions so that the ambient temperature will similarly lay between them. The shift in the  $M_d$  temperature is the primary reason for the ability to obtain high elongation at high tensile strength values.

## SUMMARY OF THE INVENTION

A primary object of this invention is to obtain a combination of high strength and high ductility in "TRIP" type steels essentially without the need for special prior mechanical deformation as required in U.S. Pat. No. 3,488,231.

Another object is to provide a method for raising the  $M_d$  of a substantially austenitic steel without the use of mechanical deformation and thereby provide for transformation of austenite to martensite under ambient temperature service conditions, resulting in a combination of greater strength and ductility.

Still another object of this invention is to provide a method for making transformation induced plasticity steels which can be welded without destroying the effects of the processing, contrary to thermomechanically processed steels, which can be used in castings of intricate shapes, and which will not necessarily be highly anisotropic.

## BRIEF SUMMARY OF THE DRAWINGS

FIG. 1 is a graph in which the ordinates are  $R_c$  hardness and the abscissae are the temperature at which the mixture of martensite and austenite was heated to cause reversion. The two curves represent two steels which contain 24% nickel and 4% molybdenum. The first steel contains 0.29% carbon and the other steel 0.22% carbon. The designation alpha on the drawing refers to martensite and the designation gamma indicates austenite in conformance with usual metallurgical practice;

FIG. 2 is an outline of the  $R_c$  hardness obtained in steel amenable to the procedure of this invention after five excursions through the thermal cycle outlined above. The martensite was formed at -320°F and the austenite by a 2 minute immersion in a salt bath at 1300°F;

FIG. 3 is similar to FIG. 2 except that it illustrates properties obtained in a sample 1/4 of an inch thick and a sample 0.060 inch thick. The reason for this difference between samples of varying thicknesses is not currently understood;

FIG. 4 is a photomicrograph at a magnification of X100 showing the steel as quenched from 1900°F. This structure is entirely austenite and has a grain size of ASTM 0;

FIG. 5 demonstrates the structure obtained after cooling to -320°F in liquid nitrogen and at a magnification of X200;

FIG. 6 shows the same steel after being reverted for 2 minutes in a salt bath at 1300°F. The sample is in excess of 99% austenite and the magnification is X200;

FIG. 7 shows the same steel after a second cooling to -320°F following a previous reversion cycle. Martensite, reverted austenite and virgin austenite are observable. The magnification again is X200;

FIG. 8 shows the final structure obtained after five reversion cycles. The magnification is again X200;

FIG. 9 has been presented to show the structure after annealing at 1900°F for 30 minutes of a sample previously cycled through five reversions. This sample is not typical of the invention. The magnification is again X200;

FIG. 10 has been presented to show the intensity vs. 2θ diffraction angle of (220) austenite peaks for the steel in the as-quenched condition, after a single reversion at 1300°F and after the fifth reversion at 1300°F;

FIG. 11 represents the stress and plastic strain of a suitable steel after various thermal processes. This drawing clearly shows the improvement in the steel as the number of reversions is increased;

FIG. 12 demonstrates the physical properties obtained after five reversions and clearly demonstrates the variation of physical properties as influenced by the reversion temperatures;

Table I is a table listing investigative results for a series of alloys from which the scope of the improvement can be proven and predicted, and

Table II is a tabulation of mechanical properties varying with thermal cycling.

#### DETAILED DESCRIPTION

A selected alloy is heated to produce a recrystallized austenite phase, then subjected to a cooling treatment to below ambient temperatures (preferably about -320°F) where about 70% of the austenite will be transformed to martensite. The selected alloy is then reheated to a temperature just above that where martensite begins to revert to austenite, but below the temperature for recrystallization into austenite. At this second stage, there is approximately 25% original austenite, 2-3% of the martensite and about 72% reverted austenite. The alloy may then be cooled to room temperature or the same thermal cycle may be repeated preferably at or above five times. The resulting steel will be substantially austenitic which transforms to martensite upon strain from a test device or by use. This method makes it possible for the first time, for an unworked austenite to be capable of transforming to martensite under such conditions.

To practice the invention successfully, it is necessary that the selected alloy meet several requirements. The steel must have an  $M_s$  below ambient temperature. The  $M_s$  is a standard metallurgical term and is defined as the temperature at which the martensite phase begins to form as the temperature is lowered. The  $M_s$  of a specimen may readily be measured by routine tests that are familiar to those skilled in the art. The  $M_d$  of the starting material must preferably be below ambient temperature. The  $M_d$  is a standard metallurgical term defined as the temperature above which the martensite phase cannot form during working of the metal. The  $M_d$  may readily be determined by standardized testing familiar to those skilled in the art. It is essential that the thermal cycling raise the  $M_d$  temperature above the expected service temperature. Lastly, the starting material must also have an austenite reversion temperature below the austenite recrystallization temperature.

The selected steel alloys used in the present investigation, which proved to be successful, substantially contained between 19.9-24.2% nickel, 2.03-4.1% molybdenum, 0-1.85% chromium, between 0.22 and 0.36% carbon, and the balance iron. However, the investigation covered alloys having an analysis range of 15.9-24.2% nickel, 2.01-6.08% molybdenum, 0-6.06% chromium, 0-1.04% manganese, 0-0.24% silicon, 0-0.97% cobalt, 0.22-0.36% carbon and the balance iron.

Turning now in some detail, the selected alloy steel is (A) normally received in the completely austenitic condition or may be processed into this condition by heating to a temperature on the order of 1800°F to 2200°F followed by a water quench. Alloy steels so quenched are essentially 100% austenitic and are relatively soft and ductile in this condition. For example, an

alloy steel having 24% nickel, 4% molybdenum, 0.2-0.3% carbon, balance Fe, had the following mechanical properties: 42,600 psi yield strength, 89,300 psi tensile strength, 38 1/2% elongation, and 80  $R_b$  (about 0  $R_c$ ) hardness. The structure of these steels remains austenitic during tensile testing indicating that the  $M_d$  is below ambient temperatures.

(B) The steel is next cooled to a temperature below  $M_s$ ; in the case of the example, the steel was cooled in liquid nitrogen to -320°F. The steel is then allowed to warm to ambient temperature. The steel is now a mixture of martensite and austenite and the example had the following mechanical properties: 119,600 psi yield strength, 155,900 tensile strength, 13% elongation and 31  $R_c$  hardness.

(C) The steel is then immersed in a liquid salt bath at a temperature above the austenite reversion temperature but below the austenite recrystallization temperature; for the steel example, it is heated in a liquid salt bath at about 1300°F for 2 minutes and air cooled to ambient temperature. This treatment causes the reversion of essentially all of the martensite to austenite; the steel had the following mechanical properties: 104,000 psi yield strength, 136,200 psi tensile strength, 36% elongation and 28  $R_c$  hardness. During tensile testing some of the austenite transformed to martensite indicating that the  $M_d$  has been increased to above ambient temperature.

The steel can be again cooled to a temperature below  $M_s$  to convert the austenitic structure to martensite and again heated to a temperature above the austenite reversion temperature but below the austenite recrystallization temperature. This procedure of cycling between martensite and austenite can be repeated until the desired mechanical properties are obtained. After five complete cycles, the reverted austenite state for the example had the following mechanical properties: 162,000 psi yield strength, 193,000 tensile strength, 30% elongation and 42 1/2  $R_c$  hardness. During tensile testing a substantial portion of the austenite transforms to martensite indicating that the  $M_d$  has been increased as compared to after the first reversion cycle.

#### Alloy Selection

For the initial experimentation related to this invention, the austenite to martensite transformation was obtained by cooling in liquid nitrogen (-320°F). One of the strongest of the prior art TRIP steels has a composition of about 9% Cr-8% Ni-4% Mo-2% Mn-2% Si-0.3% C. Unfortunately this alloy was unsatisfactory since its  $M_s$  is less than -320°F. The nominal TRIP steel composition of 24% Ni-4% Mo-0.3% C, which is the "B" alloy reported upon by Zackay, et al. was found to be useable for the initial experimentation. Two different carbon contents of this nominal composition were used as shown below:

| Designation | Composition                |
|-------------|----------------------------|
| B1          | Fe-24.2% Ni-4.1% Mo-.29% C |
| B2          | Fe-24.5% Ni-4.1% Mo-.22% C |

Following quenching from 2050°F in water to room temperature (the alloy is entirely austenitic in this condition), X-ray diffraction measurements indicated that further cooling to -320°F produced about 70% martensite in alloy B1.

The compositions listed in Table I were also investigated; alloys 1-11 proved effective in successfully being processed as alloys B1 and B2. Alloys 12-21 could not be processed according to this invention because the  $M_s$  proved to be too low (less than  $-452^{\circ}\text{F}$ ). Accordingly, an operable compositional range for the alloying ingredients of this invention was 19.9-24.5% Nickel, 2.01-4.1% Mo, up to 1.85% Cr, up to 0.25% Mn, up to 0.24% Si, and 0.22-0.36% Carbon.

#### Hardness Measurements

Samples about  $1 \times 1 \times \frac{1}{4}$  inches thick of alloys B1 and B2 were austenitized at  $2050^{\circ}\text{F}$  and water quenched. The hardness was about  $80 \text{ R}_b$  ( $\sim 0 \text{ R}_c$ ) in this condition. After cooling to  $-196^{\circ}\text{C}$  and returning to room temperature, the hardness of the martensite and austenite structure was  $31 \frac{1}{2} - 33 \text{ R}_c$ . The samples were then immersed in a salt pot at various temperatures from  $900^{\circ}$  to  $1700^{\circ}\text{F}$  for 2 minutes and air cooled to room temperature. The hardness and structure of both alloys after this heat treatment are shown in FIG. 1. The temperature for complete austenite reversion was between  $1100^{\circ}$  and  $1200^{\circ}\text{F}$ , and it was apparent that complete reversion would occur under conditions such that the austenite is appreciably harder than in the as-quenched condition. The B1 alloy that had been reverted at  $1200^{\circ}\text{F}$  was cycled through another  $-320^{\circ}\text{F}$  and  $1200^{\circ}\text{F}$  sequence, and it was noted that a duplex austenite/martensite structure then existed. The reversion temperature was evidently deemed dependent upon some structural feature that varied with continual cycling.

Another B1 sample, that had been originally reverted at  $1300^{\circ}\text{F}$ , was processed through four additional  $-320^{\circ}\text{F}$  and  $1300^{\circ}\text{F}$  cycles, and this sample was always entirely austenitic after each  $1300^{\circ}\text{F}$  treatment. FIG. 2 shows the hardness of the B1 sample that was processed through five austenite and martensite ( $-320^{\circ}\text{F}$ ) and austenite ( $1300^{\circ}\text{F}$ ) cycles after each step in the process. After the fifth reversion, the hardness of the austenite was  $42 \frac{1}{2} \text{ R}_c$ , and it appeared that the hardness was leveling off near this value.

During the course of this research, hardness readings were also made in 0.060 inch thick samples of both alloys cycled between  $-320^{\circ}\text{F}$  and  $1300^{\circ}\text{F}$ . The hardness of the austenite is shown as a function of the number of cycles in FIG. 3 for both thicknesses (0.060 inch and  $\sim \frac{1}{4}$  inch) of alloy B1, and the thinner samples are seen to be softer than the  $\frac{1}{4}$  inch thick samples. The same feature was also found in 0.060 inch and  $\sim \frac{1}{4}$  inch thick samples of alloy B2 processed through five cycles. Although an explanation for this behavior was not established, a number of variables were investigated; included in the factors that experimentally did not account for this hardness/thickness behavior are grain size, original austenitizing (solution) temperature, cooling rate down to  $-320^{\circ}\text{F}$ , time at  $320^{\circ}\text{F}$ , and time at  $1300^{\circ}\text{F}$ .

#### Metallography

The structural characteristic of the as-quenched (from  $2050^{\circ}\text{F}$ ) material from which all the previously mentioned results were obtained is shown in FIG. 4. The grain size is about ASTM 0. This material was taken from an as-forged bar where forging temperatures up to  $2250^{\circ}\text{F}$  were used; this accounts for the extremely large starting grain size.

After a single treatment at  $-320^{\circ}\text{F}$ , the duplex martensite/austenite structure appeared as shown in FIG. 5. The martensite needles reached a length that appeared to be limited by the austenite grain size. After a 2 minute reversion at  $1300^{\circ}\text{F}$ , the reverted austenite appeared as a "ghost" structure of the prior martensite as shown in FIG. 6; these "ghost" areas are seen to etch darker than the original martensite. Upon cooling to  $-320^{\circ}\text{F}$  of a once reverted sample, the martensite that formed appeared to be primarily in the virgin austenite rather than the reverted austenite. An example of the martensite, reverted austenite and virgin austenite structures is shown in FIG. 7. It might be anticipated that additional cycling would tend to convert the remaining virgin austenite to reverted austenite. This was confirmed; FIG. 8 shows the structure after the fifth reversion, and it is estimated that about 95% to 98% of the material is now reverted austenite.

In an attempt to determine whether the type of structure seen in FIG. 8 would undergo recrystallization, the sample that had been cycled through five reverisons at  $1300^{\circ}\text{F}$  was heat treated at  $1900^{\circ}\text{F}$  for 30 minutes. The resulting structure is shown in FIG. 9; in general, a considerable amount of grain refinement occurred (see FIG. 4 for the initial grain size— note difference in magnifications). The initial grain boundaries are still evident, but it is not clear whether these are real or "ghost" boundaries.

#### X-Ray Line Broadening Measurements

X-Ray diffraction measurements were made of the (220) austenite peak on alloy B1 in the as-quenched ( $2050^{\circ}\text{F}$ ) condition, after a single reversion at  $1300^{\circ}\text{F}$  and after the fifth reversion at  $1300^{\circ}\text{F}$ . The intensity vs. diffraction angle ( $2\Theta$ ) for the three conditions is shown in FIG. 10. In the as-quenched condition, the separation of the  $K \alpha_1$  and  $K \alpha_2$  peaks are readily apparent, but the broadening in both the other conditions eliminates the separation. The intensity ( $2\Theta$ ) behaviors of the reverted austenites are characteristic of that normally observed in cold worked metals.

The amount of line broadening (width of the reflection at one-half the maximum intensity) was measured in the three cases, and values of  $0.25^{\circ}$ ,  $1.20^{\circ}$ , and  $1.62^{\circ}$  were obtained for the as-quenched, the single reverted austenite, and the five cycle reverted austenite, respectively. In addition to the increase in the broadening with cycling, FIG. 10 shows that the diffraction angle corresponding to maximum intensity increases from about  $127.75^{\circ}$  ( $2\Theta$ ) for the as-quenched condition to about  $128.65^{\circ}$  after the fifth reversion. This increase in  $2\Theta$  indicates that a residual compressive stress is created by the cyclical processing.

#### Mechanical Properties

Tensile testing was done after processing of both  $\sim \frac{1}{4}$  inch and 0.060 inch thick material of alloy B1. As previously noted, the  $\sim \frac{1}{4}$  inch thick samples achieved somewhat higher hardness values than the 0.060 inch thick samples.

A 0.3 inch thick section of alloy B1 was homogenized at  $1900^{\circ}\text{F}$  and water quenched; separate tests indicated that this lower solution temperature produced equivalent hardness values through five reversion cycles. Individual samples about 0.3 inch  $\times$  0.3 inch  $\times$   $2 \frac{1}{4}$  inch were cut and given various thermal processes. All of these initial austenite to martensite transformations were done by immersing the samples in liquid nitrogen,

and all martensite to austenite transformations were done by heating for 2 minutes in a salt bath at 1300°F and air cooling. The yield strength, tensile strength, and elongation obtained with various samples are shown in FIG. 14. A single reversion is seen to increase the yield strength by about a factor of 2 1/2 without any significant loss in elongation. The primary reason for this is that during testing of the once reverted sample, the martensite transformation was induced and this promotes high elongation values for the existing flow stresses. The strain induced martensite transformation did not occur during testing of as-quenched samples. A second reversion cycle is seen to further increase the yield and tensile strength at an equivalent elongation. After the fifth reversion cycle, the yield strength has been increased by a factor of about four and the tensile strength nearly doubled with only a small loss in elongation.

Stress-strain curves for some of these samples are shown in FIG. 11. The curves for the once and twice reverted samples are characteristic of TRIP steels thermomechanically processed ~20% prior to testing. For samples processed through five reverisons, the stress-strain curve shows a yield point, Lüder's straining and work hardening stages, all of which are found in the stronger TRIP steels.

Samples of the B1 alloy 0.060 inch thick were solution treated at 1900°F and processed through five reversion cycles as a function of reversion temperatures from 1150° to 1350°F. After the fifth reversion, the samples reverted at 1150° and 1200°F consisted of a duplex martensite-austenite structure and those reverted at 1250° to 1350°F were entirely (>99%) austenitic. The yield strength, tensile strength, and elongation are shown in FIG. 12 as a function of reversion temperature. One of the most significant features of FIG. 12 is the decrease in yield strength at "reversion" temperatures where the martensite-austenite is not completed. The presence of untempered martensite also results in lower elongation values but does not appear to affect the tensile strength.

A comparison of the properties obtained in the 0.060 inch and ~1/4 inch thick samples given equivalent processing of five cyclical reverisons at 1300°F shows the following:

| Sample Thickness     | Yield Strength | Tensile Strength | Elongation |
|----------------------|----------------|------------------|------------|
| 0.060" thick samples | 142 ksi        | 184 ksi          | 27%        |
| ~1/4" thick samples  | 162 ksi        | 193 ksi          | 30%        |

The reason for this effect was not established in this initial investigation.

The normal thermomechanical processing of TRIP steels accomplishes two essential features. First, the processing must strengthen the austenite; without this processing, yield strengths of only 40–50 ksi exist. Second, the processing must raise the  $M_d$  above the testing temperature (intended service temperature). The  $M_d$  is the temperature below which the austenite and martensite transformation can be induced during plastic deformation. If a perfectly processed TRIP steel is tested above the  $M_d$  temperature, the elongation is reduced to only 1/5 to 1/10 of what can be found at temperatures below the  $M_d$ .

In the initial investigation, it is apparent that both austenite strengthening and the raising of the  $M_d$  above ambient has been established by thermal processing alone. The yield strength was increased from 42.6 ksi to 162 ksi (after five reversion cycles). Most of this strengthening is presumed to be the result of martensite (shear) transformation and is retained during the reverse transformation to austenite. Precipitation of carbides (Mo or Fe) may have contributed a minor amount to the strengthening. The comparison between carbide precipitation during thermomechanical processing and thermal processing is not known.

The change in the  $M_d$  is also thought to be related to the martensite shear transformation; the higher internal strain energy favors the austenite to martensite transformation, thus increasing the  $M_d$ . Again, however, precipitation of carbides could also have contributed some effect to the increase in  $M_d$  by changing the chemistry of the matrix.

The results clearly show that thermal processing can be used to "condition" TRIP steels. Using the results of Zackey, et al., a comparison of the mechanical properties following thermomechanical processing (80% reduction at 930°F) and thermal processing for the same alloy is shown below:

| Type of Processing                              | Yield Strength, ksi | Tensile Strength, ksi | Elongation % |
|-------------------------------------------------|---------------------|-----------------------|--------------|
| Thermomechanical<br>(80% reduction at 930°F)    | 164                 | 176                   | 41           |
| Thermal<br>(5 cycles between -320°F and 1300°F) | 162                 | 193                   | 30           |
| Thermal<br>(2 cycles between -320°F and 1300°F) | 136                 | 165                   | 36 1/2       |

It is obvious that a process consisting of 5 cycles between -320°F and 1300°F can provide the physical characteristics of a thermomechanical processing of 80% reduction at 930°F.

TABLE I

| Alloy Num- | Ni   | Mo   | Cr   | Mn  | Si  | Co | C   | Fe      |
|------------|------|------|------|-----|-----|----|-----|---------|
| <i>ber</i> |      |      |      |     |     |    |     |         |
| 1          | 24.2 | 4.1  | —    | —   | —   | —  | .29 | Balance |
| 2          | 24.5 | 4.1  | —    | —   | —   | —  | .22 | "       |
| 3          | 24.2 | 4.06 | —    | —   | —   | —  | .32 | "       |
| 4          | 23.6 | 3.85 | —    | —   | —   | —  | .36 | "       |
| 5          | 24.2 | 3.97 | —    | .25 | .24 | —  | .30 | "       |
| 6          | 21.8 | 3.79 | .96  | —   | —   | —  | .28 | "       |
| 7          | 20.2 | 3.86 | 1.78 | —   | —   | —  | .32 | "       |
| 8          | 24.0 | 2.91 | .94  | —   | —   | —  | .30 | "       |
| 9          | 23.6 | 2.01 | 1.81 | —   | —   | —  | .30 | "       |
| 10         | 21.9 | 2.96 | .96  | —   | —   | —  | .30 | "       |
| 11         | 19.9 | 2.03 | 1.85 | —   | —   | —  | .30 | "       |
| 12         | 23.9 | 6.08 | —    | —   | —   | —  | .32 | "       |

TABLE I-continued

| Alloy Num- | Ni   | Mo   | Cr   | Mn   | Si | Co  | C   | Fe |
|------------|------|------|------|------|----|-----|-----|----|
| ber        |      |      |      |      |    |     |     |    |
| 13         | 21.8 | 3.85 | 1.94 | —    | —  | —   | .32 | "  |
| 14         | 20.1 | 3.95 | 4.12 | —    | —  | —   | .32 | "  |
| 15         | 17.8 | 3.98 | 6.06 | —    | —  | —   | .31 | "  |
| 16         | 19.8 | 2.97 | 1.90 | 1.02 | —  | —   | .31 | "  |
| 17         | 17.7 | 3.04 | 4.15 | 1.03 | —  | —   | .32 | "  |
| 18         | 15.9 | 2.07 | 6.06 | 1.01 | —  | —   | .31 | "  |
| 19         | 21.8 | 3.86 | 1.94 | 1.04 | —  | .97 | .31 | "  |
| 20         | 19.9 | 3.92 | 4.11 | 1.01 | —  | .97 | .31 | "  |
| 21         | 17.9 | 3.97 | 6.02 | 1.01 | —  | .95 | .31 | "  |

TABLE II

| MECHANICAL PROPERTIES AFTER VARIOUS THERMAL PROCESSES |                         |                        |                      |                       |              |  |
|-------------------------------------------------------|-------------------------|------------------------|----------------------|-----------------------|--------------|--|
| Prior Thermal Processing                              | Structure Prior to Test | Structure After Test   | Yield Strength,* ksi | Tensile Strength, ksi | Elongation % |  |
| As-Quenched                                           | austenite               | austenite              | 42.6                 | 98.3                  | 38½          |  |
| As-Quenched Plus Liquid Nitrogen                      | martensite & austenite  | martensite & austenite | 119.6                | 155.9                 | 13           |  |
| Reverted at 1300°F                                    | austenite               | austenite & martensite | 104.4                | 136.2                 | 36           |  |
| 2 Reversion Cycles                                    | austenite               | austenite & martensite | 136.4                | 164.9                 | 36½          |  |
| 3 Reversion Cycles                                    | austenite               | austenite & martensite | 144.3                | 163.6                 | 33           |  |
| 5 Reversion Cycles                                    | austenite               | austenite & martensite | 162.0                | 193                   | 30           |  |

We claim as our invention:

1. The process of producing articles from a steel of high-strength and elongation having a metallurgical structure essentially comprised of reverted austenite, 30 by controlled heat treatment, the process comprising:

heating a steel blank to a temperature at which said blank is completely austenitic, the chemistry of said blank consisting essentially of 0.22-0.36% carbon, 19.9-24.5% Ni, 2.0-4.1% Mo and the balance 35 essentially iron, and selected to produce initial thermal martensite start temperature ( $M_s$ ) and deformation martensite start temperature ( $M_d$ ), both below ambient and an austenite reversion temperature below the temperature at which austenite recrystallizes, cooling the steel blank to produce a predominantly austenitic structure, subjecting this cooled blank to a temperature sufficiently low to transform a substantial portion of the austenite to martensite having a first level of strength, heating 40 this martensitic blank to a temperature adequate to cause a substantial portion of the martensite to revert to austenite, but at a temperature below that at which the reverted austenite recrystallizes, said reverted austenite having a first level of elongation, 45 cooling this reverted austenite blank to cause its structure to become at least partially martensitic and repeating this cycle of reverted austenite-martensite-reverted austenite until both the  $M_d$  is increased above said ambient temperature and the blank defines an article having a strength level greater than said first strength level and an elongation level at least 50 80% of said first elongation level.

2. The process recited in claim 1, in which the blank is additionally subject to strain below the final  $M_d$ , 60 thereby inducing the transformation of the reverted austenite steel to martensitic steel, whereby the strength of the strained steel is increased above the strength level resulting from said thermal cycling.

3. The process recited in claim 1, in which the blank 65 is additionally tempered in the reverted austenite.

4. A method of enhancing the strength and elongation levels of a steel through thermal cycling, comprising:

a. preparing a steel blank having a chemistry consisting essentially of 0.22-0.36% carbon, 19.9-24.5% Ni, 2.0-4.1% Mo and the balance essentially iron, and selected to provide an alloyed composition with an  $M_s$  and an  $M_d$  temperature below ambient and an austenite reversion temperature below the austenite recrystallization temperature,  
 b. austenitizing said blank and then cooling to below said  $M_s$  temperature,  
 c. subjecting said blank to at least one heating and cooling cycle wherein the blank is heated to above the austenite reversion temperature but below the austenite recrystallization temperature so that said blank is predominantly and increasingly constituted of reverted austenite, the blank is then cooled to below said  $M_s$  temperature, and  
 d. in the final cooling step, limiting said cooling to above the  $M_s$  temperature.

5. The process of producing a steel of high strength and high elongation having a metallurgical structure essentially comprised of reverted austenite, by controlled heat-treatment the steel being particularly characterized in that it has a thermal martensite starting temperature ( $M_s$ ) well below ambient temperature and the lowest anticipated service temperature, and a deformation martensite start temperature ( $M_d$ ), also below the ambient temperature, and an austenite reversion temperature below the austenite recrystallization temperature, said steel consisting essentially of 0.22-0.36% carbon, 19.9-24.5% Ni, 2.0-4.1% Mo and the balance essentially iron being subjected to the following heat treatment:

a. heating the steel to a temperature at which the steel is completely austenitic,  
 b. cooling said steel to a temperature below said ( $M_s$ ) to provide a predominantly martensitic steel structure,  
 c. heating said predominantly martensitic steel to a temperature above said austenite reversion temperature but below said austenite recrystallization temperature to provide a structure predominantly of reverted austenite, and

d. cooling this steel with its predominantly reverted austenite structure being retained, repeating said heat-treatment cycle of transformation from austenitic via martensitic to reverted austenitic structure.

6. The process as in claim 5, in which said repetition of said heat treatment is carried out to provide an increase in the  $M_a$  over the starting value, and also to

provide said steel with a strength exceeding that of the steel as obtained from the first cooling step (b) and an elongation at least 80% of the elongation of the steel as obtained from the first step (c).

5 7. The process as in claim 5, in which the reversion temperature is at about 1300°F.

\* \* \* \* \*

10

15

20

25

30

35

40

45

50

55

60

65